

3,560,174

## MOTOR FUEL COMPOSITION

Stanley R. Newman, Fishkill, Kenneth L. Dille, Wappingers Falls, and Rodney L. Sung, Fishkill, N.Y., assignors to Texaco Inc., New York, N.Y.

No Drawing. Filed Nov. 22, 1967, Ser. No. 684,971  
Int. Cl. C011 1/26

U.S. Cl. 44—69

4 Claims

### ABSTRACT OF THE DISCLOSURE

Motor fuel composition containing 2-chloroethyl diphenyl phosphate surface ignition suppressor.

This invention relates to a motor fuel composition for spark-ignited internal combustion engines. More particularly, this invention relates to a motor fuel composition having improved surface ignition properties based on a phosphate ester additive.

Organic phosphorus compounds have been proposed for use in motor fuel compositions for various purposes, such as load-carrying additives, scavengers, surface ignition suppressors and the like, see U.S. 2,291,442, U.S. 2,889,212 and U.S. 2,892,691. Despite extensive art disclosing advantages from the use of organic phosphate additives, their commercial adoption has been restricted to a few types of phosphorus compounds largely because of the anti-knock destruction values associated with most phosphorus additives. That these values are high is shown in an article entitled "The Effect of Phosphorus Deposit Modifiers on Gasoline Octane Quality" by Gunderloy and Neblett, which appeared in a paper presented to the Petroleum Chemistry Division of the American Chemical Society given at Cleveland, Ohio on April 5-14, 1960, pages 75 to 86. On page 85, of this paper, there are examples of organic phosphorus additives, such as tributyl phosphate, dibutyl phosphate and tributyl phosphine, which had anti-knock destruction values ranging from -1.5 to -3.6 as determined by the Motor Octane Number method. When it is realized that an increase of but 0.1 Motor Octane Number in a modern high-octane gasoline is an important and valuable improvement, it is evident that anti-knock destruction values of the order noted are prohibitive.

An organic phosphorus compound additive for gasoline has now been discovered which is highly effective for improving the surface ignition properties of a high octane gasoline while at the same time exhibiting an unexpectedly low anti-knock destruction value.

In accordance with this invention, there is provided a motor fuel composition comprising a mixture of hydrocarbons in a gasoline boiling range containing from about 0.1 to 1.0 theory of 2-chloroethyl diphenyl phosphate. The expression "theory" as used herein relates to the amount of phosphorus required to react stoichiometrically with the lead present in the gasoline to form  $Pb_3(PO_4)_2$ . The preferred amount of the surface ignition suppressor is from 0.2 to 0.5 theory.

The surface ignition additive of the invention is added to a motor fuel in the gasoline boiling range containing an anti-knock amount of an alkyllead compound. The motor fuel may consist of any hydrocarbon fuel including paraffinic, naphthenic and aromatic hydrocarbons or mixtures thereof, suitable for use in spark-ignited internal-combustion engine. These fuels are obtained from the distillation of crude oil, by the catalytic or thermal cracking of gas oils, by the alkylation of isoparaffins with olefins, or by the polymerization of olefins. The boiling point of the motor fuel or gasoline will generally be in the range from 100° F. to about 400° F. The motor fuel

of the invention will contain a tetraalkyl lead compound, such as tetraethyl lead or tetramethyl lead, in a concentration ranging from about 0.5 ml. to about 4 ml. per gallon of fuel. The motor fuel may also contain a number of additives conventionally employed in gasoline, such as anti-oxidants, stabilizers, dyes, and metal suppressors.

A gasoline containing the additive of the invention was tested for its surface ignition effectiveness in an 11.3/1 compression ratio cylindrical wedge single cylinder engine. The engine was continuously run on the test fuel over a 20-hour test period during which time the engine operation was alternated between a 50-second idle cycle (600 r.p.m.) and a 150-second full throttle cycle (900 r.p.m.). The surface ignition count rate was obtained using an ionization gap (spark plug) as a surface ignition pick-up coupled to a recording counter device. The surface ignition rate is expressed as the number of counts per hour, the lower the count value the better the surface ignition performance of the fuel.

20 The tests were conducted using a high octane blended gasoline as the base motor fuel. This gasoline contained 41% aromatic hydrocarbons, boiled in the range of 95 to 354° F., had a motor octane number of 91.3 and contained 3 ml. of TEL per gallon. The additive of the invention was blended into this leaded gasoline to provide the indicated amounts of phosphorus in theories. The results are the average of three runs.

The base fuel was found to give 190 surface ignition counts per hour.

30 At a concentration of 0.2 theory 2-chloroethyl diphenyl phosphate in the additive-containing fuel, this fuel was found to give 145 surface ignition counts per hour. This performance is a substantial improvement in surface ignition properties as compared to the surface ignition properties of the base fuel.

35 As indicated above, the critical factor which prohibits the use of most organic phosphorous compounds in gasoline is the high anti-knock losses caused by these additives. A surface ignition additive having an AKD (anti-knock destruction) value greater than zero requires the addition of extra tetraethyl lead or other anti-knock additives to bring the gasoline up to its original anti-knock quality, thus imposing a severe economic penalty.

The AKD caused by the additive of the invention and 45 by a related organic phosphate was determined using the motor octane number method. The base fuel was a 100 RON premium leaded gasoline containing 3.0 ml. of tetraethyl lead and having a motor octane number of 89.4. The organic phosphate additives were employed at concentrations of 0.2 and 0.4 theories of phosphorus. The octane determinations were made by an absolute number method in which engine, operator and time variables were controlled by each set of determinations. Three or more series were averaged and compared to the base fuel without the 50 phosphorus additive present.

### Anti-Knock Destruction Values for Additives by the Motor Octane Method

|            |                                                | ΔMON        |
|------------|------------------------------------------------|-------------|
| 60         | 0.2 theory<br>2-chloroethyl diphenyl phosphate | ----- +0.03 |
|            | Tris-2-chloroethyl phosphate                   | ----- -0.5  |
| 0.4 theory |                                                |             |
|            | 2-chloroethyl diphenyl phosphate               | ----- -0.1  |
|            | Tris-2-chloroethyl phosphate                   | ----- -0.5  |

65 It is evident that the anti-knock destruction value of 2-chloroethyl diphenyl phosphate is a vast improvement over that of the other halogenated phosphate ester, tris-2-chloroethyl phosphate. 2-chloroethyl diphenyl phosphate is a satisfactory commercial additive from the standpoint 70 of the critical anti-knock destruction value as well as for surface ignition improvement in contrast to the unacceptable tris-2-chloroethyl phosphate.

Obviously, many modifications and variations of the invention, as hereinafter set forth, may be made without departing from the spirit and scope thereof, and therefore, only such limitations should be imposed as are indicated in the appended claims.

We claim:

1. A motor fuel composition comprising a mixture of hydrocarbons in the gasoline boiling range containing a tetraalkyl lead anti-knock additive and from about 0.1 to 1 theory of 2-chloroethyl diphenyl phosphate.

2. A motor fuel composition according to claim 1 in which said phosphate is employed in a concentration of 0.2 to 0.5 theory.

3. A motor fuel composition according to claim 1 con-

taining from about 0.5 to 4 ml. per gallon of tetraalkyl lead anti-knock agent.

4. A motor fuel composition according to claim 3 containing tetraethyl lead.

**References Cited**

**UNITED STATES PATENTS**

2,892,691 6/1959 Howell, Jr. ----- 44-69P

10 PATRICK P. GARVIN, Primary Examiner

Y. H. SMITH, Assistant Examiner

U.S. Cl. X.R.

44-69P, 76